

## UNITED STATES PATENT OFFICE

2,322,959

## TANNING

Herbert J. West, Old Greenwich, Conn., assignor  
to American Cyanamid Company, New York,  
N. Y., a corporation of Maine

No Drawing. Application October 25, 1941,  
Serial No. 416,493

## 8 Claims. (Cl. 149—5)

This invention relates to the treatment of hides and more particularly to the production of white tanned leathers.

According to the present invention, tanning of hides for the production of white leathers may be accomplished by impregnating the hides with an aqueous solution of a water-soluble dialkyl ether of dimethylol urea and acidifying the impregnated hides to set or resinify the contained dialkyl ether.

As white tanning agents, any water soluble diether of a monohydric aliphatic alcohol and dimethylol urea may be employed, for example, the dimethyl, di-ethyl, di-n-propyl, di-iso-propyl and di(ethylene glycol monoalkyl ether) ethers of dimethylol urea. For purposes of the present invention, the crystalline form of the dimethylol urea ethers is preferred, although in some instances the syrupy partially dealkylated dialkyl ethers may likewise be employed. These syrupy products may be obtained by heat treatment of the crystalline diethers in the presence of small quantities of an acid the dissociation constant of which is greater than  $1 \times 10^{-5}$ , e. g., oxalic, phosphoric acids, etc.

It is an advantage of the process of the present invention that white leathers may be obtained which are fully light fast, give no color reaction with salts of iron and from which the tanning agent is not extractable with water or with dilute acids or alkalies.

In the practice of the invention, the hides to be tanned are drummed in an aqueous solution of sodium chloride and one of the water-soluble dialkyl ethers of dimethylol urea. The drumming is continued until a thorough penetration of the hides with the solution of the dialkyl ether has been effected. The impregnated hides are then acidified by the gradual addition of dilute acid thereto followed by drumming, the acid being preferably added to the hides when present in the tanning bath. Following the acidification, the hides are preferably removed from the drum and allowed to stand for several hours or over night to give the acid additional time to cause setting or resinification of the contained dialkyl ether. The acidity of the hides is then reduced with a dilute solution of sodium bicarbonate applied in the manner customary for neutralizing hides, following which the hides are washed and drained. The tanned hides may then be fatliquored in the usual manner.

The application of the dialkyl ethers of dimethylol urea in the white tanning of hides is

illustrated by the following specific example in which parts are by weight.

## Example 1

- 5        3000 parts of pickled goat skin (3 skins) were drummed for two hours in an aqueous tanning bath composed of 3000 parts of a 10% sodium chloride solution and 300 parts of the dimethyl ether of dimethylol urea previously dissolved in water. To the tanning bath was then gradually added about 600 parts of dilute sulfuric acid (10%) and the skins drummed for 3½ hours, left in the bath overnight, drummed for five minutes, and drained. To the drained skins was 10 added 6000 parts of 10% sodium chloride solution, drumming resumed, and the acidity of the skins reduced to pH 3.8-4.0 by the gradual addition to the bath of 600 parts of 10% sodium bicarbonate solution. The skins were then drummed for four 15 hours, drained, and removed from the drum. Two of the tanned skins were washed in cold running water for fifteen minutes, drained, fatliquored in the usual manner, set out and dried. The leather was white, full, and well-tanned.
- 20        While in the above example 10% of the dialkyl ether of dimethylol urea on the drained pickled weight of the hides was employed, the quantity of the dialkyl ether may be varied depending upon the weight of the hide to be tanned, the heavier 25 hides requiring more of the dialkyl ether and also a longer drumming time, as will be understood by those skilled in the art.
- In place of sulfuric acid, any other sufficiently strong acid may be employed in dilute solution 30 for setting or resinifying the dialkyl ether contained in the hides, for example, hydrochloric, phosphoric, formic, lactic, alpha-hydroxy-isobutyric, gluconic, citric, oxalic, tartaric, maleic, succinic acids, etc.
- 35        In applying the water-soluble dialkyl ethers of dimethylol urea in the tanning process, they are preferably first dissolved in water to form a solution thereof before addition to the tanning bath. In some instances it may be found preferable or even necessary to dissolve the dialkyl ethers in hot water, particularly where they are but slightly soluble in cold water. The solubility of the ethers is, in general, inversely proportional to the length of the carbon chain of the alkyl group, the longer the chain the lower the water 40 solubility of the dialkyl ether.
- The leathers obtainable by the process of the present invention may be subjected to further tanning by suitable processes, e. g., formaldehyde, alum, chrome, and vegetable tanning. The white 45

tanning process of the present invention may also be applied for the retanning of leathers, for example, to the retanning of formaldehyde, alum, chrome or vegetable tanned leathers.

*Example 2*

The remaining white tanned skin from Example 1 was subjected to formaldehyde tannage in the known manner using 5% of formaldehyde on the drained pickled weight of the skin. The retanned skin showed an increase in heat resistance over the tanned skins of Example 1.

The retanned skin was then washed, fatliquored in the usual manner, set out and dried. The leather was white, full and excellently tanned.

While the process has been more particularly described with reference to the tanning of pickled stock, it may be applied in similar manner to the white tanning of depickled and bated hides, suitable adjustment being made in the quantity of acid employed.

The dialkyl ethers of dimethylol urea may be prepared by known methods or by the procedure described in my co-pending application, Serial No. 404,203, filed July 26, 1941.

Since suitable variations and changes may be made in the invention without departing from the spirit and scope thereof, the foregoing description is intended by way of illustration except as may be defined in the appended claims.

I claim:

1. In the tanning of hides to make leather, the steps which comprise impregnating the hide with an aqueous solution of a diether of a monohydric aliphatic alcohol and dimethylol urea and acidifying the hide to resinify the ether contained therein.

2. In the tanning of hides to make leather, the steps which comprise impregnating the hide with an aqueous solution of the dimethyl ether of dimethylol urea and acidifying the hide to resinify the ether contained therein.

3. In the tanning of hides to make leather, the steps which comprise impregnating the hide with an aqueous solution of the diethyl ether of dimethylol urea and acidifying the hide to resinify the ether contained therein.

4. In the tanning of hides to make leather, the steps which comprise impregnating the hide with an aqueous solution of a dipropyl ether of dimethylol urea and acidifying the hide to resinify the ether contained therein.

5. Leather tanned with a water-soluble diether of a monohydric alcohol and dimethylol urea and containing the same in resinified form non-extractable with water or with dilute acids or alkalies, said leather being obtainable by the process of claim 1.

6. Leather tanned with the dimethyl ether of dimethylol urea and containing the same in resinified form non-extractable with water or with dilute acids or alkalies, said leather being obtainable by the process of claim 2.

7. Leather tanned with the diethyl ether of dimethylol urea and containing the same in resinified form non-extractable with water or with dilute acids or alkalies, said leather being obtainable by the process of claim 3.

8. Leather tanned with a dipropyl ether of dimethylol urea and containing the same in resinified form non-extractable with water or with dilute acids or alkalies, said leather being obtainable by the process of claim 4.

HERBERT J. WEST.